

## UNITED STATES PATENT OFFICE.

JOHN HARRIS, OF CLEVELAND, OHIO.

## GASEOUS FUEL.

No Drawing.

Application filed December 6, 1923. Serial No. 678,808.

This invention relates to gaseous fuels, and more particularly to a gaseous fuel which, when used in combination with oxygen, is especially adapted for the purpose 5 of cutting metals.

It is the general object of the invention to produce a gaseous fuel which is relatively inexpensive, which will enable the cutting operation to be performed in a most efficient 10 manner, and with the use of a gas which is ordinarily readily obtainable.

I prepare a gaseous fuel by which the foregoing general object may be realized by saturating or impregnating artificial 15 illuminating gas with ordinary commercial ether. The most convenient manner in which this saturation or impregnation may be accomplished is by introducing into a cylinder containing about 200 cu. ft. of artificial 20 gas, from one to two pounds of commercial ether. When the delivery valve from such a tank is opened, the artificial gas, impregnated with the ether, will be supplied to the blowpipe and the latter may be operated 25 with oxygen in the usual manner. When the ether is added to and mixed with the artificial illuminating gas in the manner set forth hereinbefore, the resultant gaseous fuel will consist of approximately 97½ 30 to 95 parts by volume of such gas, to approximately 2½ to 5 parts by volume of ether vapor.

The advantage of my fuel mixture is that the ether increases the flame temperature 35 and the heat units of the artificial gas, both of which are lower than in the case of acetylene. Furthermore, by reason of the fact that it lowers the igniting point of the illuminating gas which is high as compared 40 with that of acetylene and other cutting gases, the mixture can be used with ordinary blowpipe tips, without danger of the flame being blown off such tips, as is the case where artificial gas is attempted to be 45 used without dilution with such heavier hydrocarbon as then tips intended for burning illuminating gas have to be provided with special cups for the prevention of this blowing out or blowing off of the preheat- 50 ing flame.

By the use of my invention, the artificial illuminating gas can now be used with the

same facility as ordinary cutting gases, but at much less cost and with greater efficiency.

Where one pound of ether is employed 55 with a cylinder of gas, the resultant gas will realize all of the advantages set forth hereinbefore; where two pounds of ether are employed with a cylinder of gas, a corresponding increase in flame temperature and 60 heat units will be realized, with a corresponding increase in the speed of cutting, and the igniting point will be further lowered, thus insuring the maintenance of the flame at the blowpipe tips without liability 65 of being blown off. Furthermore, with the higher limit or larger quantity of ether, the gas is particularly useful for cutting heavy 70 masses of metal or dirty metal with great facility.

While commercial or ethyl ether is preferred for admixture with artificial gas, because of its richness in carbon and hydrogen, my invention contemplates the use of methyl ether, as well, for such admixture. 75

The artificial illuminating gas referred to herein is a coal gas of approximately the following composition:

|                 | Percentage by volume. |
|-----------------|-----------------------|
| CO <sub>2</sub> | 2                     |
| Illuminants     | 4                     |
| O <sub>2</sub>  | 0.5                   |
| CO              | 8                     |
| H <sub>2</sub>  | 47                    |
| CH <sub>4</sub> | 32                    |
| N <sub>2</sub>  | 6.5                   |

Having thus described my invention, what I claim is:—

1. A cutting gas consisting of a gas having a high igniting point, and having mixed therewith vapor of ether, said vapor constituting not materially less than 2½ parts and not materially more than 5 parts by volume of the mixture.

2. A cutting gas consisting essentially of 95 artificial illuminating gas having mixed therewith vapor of ether, said vapor constituting not materially less than 2½ parts and not materially more than 5 parts by 100 volume of the mixture.

In testimony whereof, I hereunto affix my signature.

JOHN HARRIS.